

## [54] DUAL TEMPERATURE COAL SOLVATION PROCESS

3,645,885 2/1972 Harris et al. .... 208/8  
3,808,119 4/1974 Bull et al. .... 208/8

[75] Inventors: **Charles H. Wright**, Overland Park, Kans.; **Gerald R. Pastor**, Takoma, Wash.

*Primary Examiner*—Delbert E. Gantz  
*Assistant Examiner*—James W. Hellwege

[73] Assignee: **The United States of America as represented by the Secretary of the Interior**, Washington, D.C.

[22] Filed: **Mar. 4, 1974**

[21] Appl. No.: **446,971**

[52] U.S. Cl. .... **208/8**

[51] Int. Cl. .... **C10g 1/00**

[58] Field of Search ..... 208/8

## [56] References Cited

## UNITED STATES PATENTS

3,341,447 9/1967 Bull et al. .... 208/8  
3,594,304 7/1971 Seitzer et al. .... 208/8

## [57] ABSTRACT

A solvation process for producing deashed solid and liquid hydrocarbonaceous fuel from coal. Raw coal is slurried with a solvent comprising hydroaromatic compounds in contact with hydrogen in a first zone at a relatively high temperature to dissolve hydrocarbonaceous fuel from coal minerals by transfer of hydrogen from hydroaromatic solvent compounds to hydrocarbonaceous material in the coal. The solvent is then treated with hydrogen in a second zone at a lower temperature to replenish the solvent with hydrogen. Forced cooling of the slurry between zones accomplishes many significant improvements in the process.

15 Claims, 7 Drawing Figures

FIG. 2



FIG. 1



FIG. 4



FIG. 3



FIG. 6



FIG. 5



FIG. 7



## DUAL TEMPERATURE COAL SOLVATION PROCESS

This invention resulted from work performed under Contract No. 14-01-0001-496 between The Pittsburgh and Midway Coal Mining Co., a subsidiary of Gulf Oil Corporation, and the Office of Coal Research in the Department of the Interior entered into pursuant to the Coal Research Act, 30 USC 661 to 668.

This invention relates to a non-catalytic liquid solvent dissolving process for producing reduced or low ash hydrocarbonaceous solid fuel and hydrocarbonaceous distillate liquid fuel, from ash-containing raw coal. Preferred coal feeds contain hydrogen, such as bituminous and sub-bituminous coals, and lignites. The process produces deashed solid fuel (dissolved coal) together with as much coal derived liquid fuel as possible, with an increase in liquid fuel product being accompanied by a decrease in solid fuel product. Liquid fuel is the more valuable product but the production of liquid fuel is limited because it is accompanied by production of undesired by-product hydrocarbon gases. Although liquid fuel is of greater economic value than deashed solid fuel, hydrocarbon gases are of smaller economic value than either deashed solid fuel or liquid fuel and have a greater hydrogen to carbon ratio than either solid or liquid fuel so that their production is not only wasteful of other fuel product but is also wasteful of hydrogen.

Hydrocarbon gases are produced primarily by hydrocracking, and since their production is undesired in this process no external catalyst is employed, since catalysts generally impart hydrocracking activity in a coal solvation process.

When raw coal is subjected to solvation at a relatively low temperature, the dissolved product comprises in major proportion a high molecular weight fuel which is solid at room temperature. When the mixture of solvent and dissolved coal is subsequently filtered to remove ash and undissolved coal and the filtrate is then subjected to vacuum distillation, this high boiling solid fuel product is recovered as the vacuum bottoms. This deashed vacuum bottoms product is referred to herein as either vacuum bottoms or deashed solid fuel product. This vacuum bottoms is cooled to room temperature on a conveyor belt and is scraped from the belt as fragmented deashed hydrocarbonaceous solid fuel.

As the temperature of the solvation process is progressively increased, the vacuum bottoms (deashed solid fuel), which is a high molecular weight polymer, is converted to lower molecular weight hydrocarbonaceous liquid fuel which is chemically similar to the process solvent and which has a similar boiling range. The liquid fuel product is in part recycled as process solvent for the subsequent pass and is referred to herein as either liquid fuel product or excess solvent. Production of liquid fuel occurs by depolymerization of solid fuel through various reactions, such as removal therefrom of heteroatoms, including sulfur and oxygen. As a result of the depolymerization reactions, the liquid fuel has a somewhat higher hydrogen to carbon ratio than the solid fuel and therefore exhibits a correspondingly higher heat content upon combustion. It is desirable in the process to convert as much of the vacuum bottoms (solid fuel) product to solvent boiling range (liquid fuel) product, since liquid fuel is economically more valuable than solid fuel. As the temperature of

solvation continues to be increased, an increasing proportion of vacuum bottoms fuel is converted to solvent boiling range fuel until a temperature is reached at which conversion of vacuum bottoms to liquid fuel occurs only at the price of excessive and wasteful production of relatively hydrogen-rich by-product hydrocarbon gases due to the onset of excessive thermal hydrocracking. The present process produces 20 or 40 to 80 weight percent of deashed solid fuel on an MAF (moisture and ash free) basis, the remaining product being primarily liquid fuel.

It is the purpose of the present invention to avoid thermal hydrocracking as much as possible and at least to the extent of avoiding excessive production of hydrocarbon gases since production of gases diminishes the yield of desired deashed solid fuel and liquid fuel products. This purpose is accomplished according to the present invention by performing the solvation process in two separate stages, each stage employing a different temperature. In one embodiment of this invention, less than 6 weight percent of hydrocarbon gases, based on MAF coal feed, is produced. The production limit of hydrocarbon gases establishes the production limit of liquid fuel product and therefore also the production limit of solid fuel product.

A further and very important advantage of the dual temperature method of this invention is that a high temperature stage is made possible whereby product sulfur level can be reduced. Relatively high temperatures are required for sulfur removal whereas temperatures below the required level are not as effective for sulfur removal. The high temperatures required for effective sulfur removal also induce hydrocracking but the hydrocracking reaction is more time dependent and by rapid reduction of the high process temperature reduction of sulfur level is achieved with a minimum of hydrocracking.

The first reactor stage of the present process is a tubular preheater having a relatively short residence time in which a slurry of feed coal and solvent in essentially plug flow is progressively increased in temperature as it flows through the tube. The tubular preheater has a length to diameter ratio of at least 100, generally and at least 1,000, preferably. A series of different reactions occur within a flowing stream increment as the temperature of the increment increases from a low inlet temperature to a maximum or exit temperature, at which it remains for only a short time. The second reactor stage employs a relatively longer residence time in a larger vessel maintained at a substantially uniform temperature throughout. An important feature of this invention is that a regulated amount of forced cooling occurs between the stages so that the second stage temperature is lower than the maximum preheater temperature. Although the preheater stage is operated with plug flow without significant backmixing, full solution mixing with a uniform reactor temperature occurs in the dissolver stage. Data presented below show that the split temperature coal dissolving process of this invention results in high conversion of raw coal to deashed solid fuel and liquid fuel and the proportion of liquid to solid fuel product is enhanced while avoiding excessive production of by-product hydrocarbon gases. It is shown below that these results are better accomplished by employing a split temperature process than by employing a process having a uniform temperature in the two stages, even when the uniform temperature is the

same as either temperature of a split temperature operation.

The coal solvent for the present process comprises liquid hydroaromatic compounds. The coal is slurried with the solvent for charging to the first or preheater stage. In the first stage, hydrogen transfer from the solvent hydroaromatic compounds to coal hydrocarbonaceous material occurs resulting in swelling of the coal and in breaking away of hydrocarbon polymers from coal minerals. The range of maximum temperatures suitable in the first (preheater) stage is generally 400° to 525°C., or preferably 425° to 500°C. If there is inadequate facilities to handle hydrocarbon gaseous by-products, the upper temperature limit should be 470°C., or below in order to minimize production of gaseous product. The residence time in the preheater stage is generally 0.01 to 0.25 hours, or preferably 0.01 to 0.15 hours.

In the second (dissolver) stage of the process of this invention, the solvent compounds, which have been depleted of hydrogen and converted to their precursor aromatics by hydrogen donation to the coal in the first stage, are reacted with gaseous hydrogen and reconverted to hydroaromatics for recycle to the first stage. The temperature in the dissolver stage is 350° to 475°C., generally, and 400° to 450°C., preferably. The residence time in the dissolver stage is 0.1 to 3.0 hours, generally, and 0.15 to 1.0 hours, preferably. The temperature in the dissolver stage is lower than the maximum temperature in the preheater stage. Any suitable forced cooling step can be employed to reduce stream temperature between the preheater and the dissolver. For example, makeup hydrogen can be charged to the process between the preheater and dissolver steps or a heat exchanger can be employed. Also, the residence time in the preheater is lower than the residence time in the dissolver.

The liquid space velocity for the process (volume of slurry per hour per volume of reactor) ranges from 0.2 to 8.0, generally, and 0.5 to 3.0, preferably. The ratio of hydrogen to slurry ranges from 200 to 10,000 standard cubic feet per barrel, generally, and 500 to 5,000 standard cubic feet per barrel, preferably, (3.6 to 180, generally, and 9 to 90, preferably, SCM/100L). The weight ratio of recycled solvent product to coal in the feed slurry ranges from 0.5:1 to 5:1, generally, and from 1.0:1 to 2.5:1, preferably.

The reactions in both stages occur in contact with gaseous hydrogen and in both stages heteroatom sulfur and oxygen are removed from solvated deashed coal polymers, resulting in depolymerization and conversion of dissolved coal polymers to desulfurized and deoxygenated free radicals of reduced molecular weight. These radicals radical have a tendency to repolymerize at the high temperatures reached in the preheater stage, but at the reduced temperature of the dissolver stage of this invention these free radicals tend to be stabilized against repolymerization by accepting hydrogen at the free radical site. The present process can employ carbon monoxide and steam together with or in place of hydrogen since carbon monoxide and steam react to form hydrogen. The steam can be derived from feeding wet coal or can be injected as water. The reaction of hydrogen at the free radical site occurs more readily at the relatively low dissolver temperature than at the higher preheater exit temperature.

The solvent used at process start-up is advantageously derived from coal. Its composition will vary, depending on the properties of the coal from which it is derived. In general, the solvent is a highly aromatic liquid obtained from previous processing of fuel, and generally boils within the range of about 150°C. to 450°C. Other generalized characteristics include a density of about 1.1 and a carbon to hydrogen mole ratio in the range from about 1.0 to 0.9 to about 1.0 to 0.3. 5 Any organic solvent for coal can be used as the start-up solvent in the process. A solvent found particularly useful as a start-up solvent is anthracene oil or creosote oil having a boiling range of about 220°C. to 400°C. However, the start-up solvent is only a temporary process 10 component since during the process dissolved fractions of the raw coal constitute additional solvent, which, when added to start-up solvent, provides a total amount of solvent exceeding the amount of start-up solvent. Thus, the original solvent gradually loses its identity 15 and approaches the constitution of the solvent formed by solution and depolymerization of the coal in the process. Therefore, in each pass of the process after start-up, the solvent can be considered to be a portion of the liquid product produced in previous extraction of the 20 raw coal.

The residence time for the dissolving step in the preheater stage is critical in the process of this invention. Although the duration of the solvation process can vary for each particular coal treated, viscosity changes as 25 the slurry flows along the length of the preheater tube provide a parameter to define slurry residence time in the preheater stage. The viscosity of an increment of feed solution flowing through the preheater initially increases with increasing increment time in the preheater, followed by a decrease in viscosity as the solubilizing of the slurry is continued. The viscosity would rise again at the preheater temperature, but preheater residence time is terminated before a second relatively large increase in viscosity is permitted to occur. An advantageous means for establishing proper time for completion of the preheater step is use of the "Relative Viscosity" of the solution formed in the preheater, which is the ratio of the viscosity of the solution formed to the viscosity of the solvent, as fed to the process, both viscosities being measured at 99°C. Accordingly, the term 30 "Relative Viscosity" as used herein is defined as the viscosity at 99°C., of an increment of solution, divided by the viscosity of the solvent alone fed to the system 35 measured at 99°C., i.e.

40 50 
$$\text{Relative Viscosity} = \text{Viscosity of Solution at } 99^\circ\text{C.} / \text{Viscosity of Solvent at } 99^\circ\text{C.}$$

The "Relative Viscosity" can be employed as an indication of the residence time for the solution in the preheater. As the solubilizing of an increment of slurry 45 proceeds during flow through the preheater, the "Relative Viscosity" of the solution first rises above a value of 20 to a point at which the solution is extremely viscous and in a gel-like condition. In fact, if low solvent to coal ratios are used, for example, 0.5:1, the slurry 50 would set up into a gel. After reaching the maximum "Relative Viscosity," well above the value of 20, the "Relative Viscosity" of the increment begins to decrease to a minimum, after which it has a tendency to again rise to higher values. The solubilization proceeds 55 until the decrease in Relative Viscosity (following the initial rise in Relative Viscosity) falls to a value at least 60 below 10, whereupon the preheater residence time is 65

terminated and the solution is cooled and passed to the dissolver stage which is maintained at a lower temperature to prevent the Relative Viscosity from again rising above 10. Normally, the decrease in Relative Viscosity will be allowed to proceed to a value less than 5 and preferably to the range of 1.5 to 2. The conditions in the preheater are such that the Relative Viscosity will again increase to a value above 10, absent abrupt termination of preheater exit conditions, such as a forced lowering of temperature.

When a slug of hydroaromatic solvent and coal first experience heating in the preheater, the first reaction product is a gel which is formed in the temperature range 200° to 300°C. Formation of the gel accounts for the first increase in Relative Viscosity. The gel forms due to bonding of the hydroaromatic compounds of the solvent with the hydrocarbonaceous material in the coal and is evidenced by a swelling of the coal. The bonding is probably a sharing of the solvent hydroaromatic hydrogen atoms between the solvent and the coal as an early stage in transfer of hydrogen from the solvent to the coal. The bonding is so tight that in the gel stage the solvent cannot be removed from the coal by distillation. Further heating of a slug in the preheater to 350°C. causes the gel to decompose, evidencing completion of hydrogen transfer, producing a deashed solid fuel, liquid fuel and gaseous products and causing a decrease in Relative Viscosity.

A decrease of Relative Viscosity in the preheater is also caused by depolymerization of solvated coal polymers to produce free radicals therefrom. The depolymerization is caused by removal of sulfur and oxygen heteroatoms from hydrocarbonaceous coal polymers and by rupture of carbon-carbon bonds by hydrocracking to convert deashed solid fuel to liquid fuel and gases. The depolymerization is accompanied by the evolution of hydrogen sulfide, water, carbon dioxide, methane, propane, butane, and other hydrocarbons.

At the high temperatures of the preheater outlet zone, repolymerization of free radicals is a reaction which is favored over hydrogenation of free radical sites and accounts for the final tendency towards increase in Relative Viscosity in the preheater to a value above 10. This second increase in Relative Viscosity is avoided in accordance with the present invention. The elimination of sulfur and oxygen from the solvated deashed solid fuel is probably caused by stripping out of these materials by thermal rupture of bonds leaving free radical molecular fragments which have a tendency towards subsequent repolymerization at elevated temperature conditions. The drop in stream temperature by forced cooling following the preheater step in accordance with this invention tends to inhibit polymer formation. The observed low level of sulfur in the liquid fuel product, which for one coal feed is about 0.3 weight percent, as compared to 0.7 weight percent in the vacuum bottoms (solid fuel) product, indicates that sulfur is being stripped out of the solid fuel product leaving low sulfur smaller molecular fragments as free radicals.

We have found that maximum or exit preheater temperatures should be in the range of 400° to 525°C. The residence time in the preheater for a feed increment to achieve this maximum temperature is about 0.01 to 0.25 hours. At this combination of temperature and residence time, coke formation is not a problem unless flow is stopped, that is, unless the residence time is in-

creased beyond the stated duration. The hydrocarbon gas yield under these conditions is less than about 6 weight percent while excess solvent (liquid fuel) yield is above 10 or 15 weight percent, based on MAF coal feed, while the solid fuel product is above 20 weight percent. High production of gases is to be avoided because such production involves high consumption of hydrogen and because special facilities are required. However, a gaseous yield above 6 weight percent can be tolerated if facilities to handle or store and transport the gas are available.

The relatively low sulfur content in the vacuum bottoms (deashed solid fuel) product of the present process is an indication that the reaction proceeds to a high degree of completion. It is also an indication that the vacuum bottoms product has been chemically released from the ash so that it can be filtered therefrom.

The hydrogen pressure in the present process is 35 to 300 kg/cm<sup>2</sup>, generally, and 50 to 200 kg/cm<sup>2</sup>, preferably. At about 70 kg/cm<sup>2</sup> hydrogen pressure, the solvent hydrogen content tends to adjust to about 6.1 weight percent. If the hydrogen content of the solvent is above this level, transfer of hydroaromatic hydrogen to the dissolved fuel tends to take place, increasing production of liquid fuel, which has a higher hydrogen content than solid fuel. If the solvent contains less than 6.1 weight percent of hydrogen, the solvent tends to acquire hydrogen from hydrogen gas at a faster rate than the fuel product. Once the solvent is roughly adjusted to a stable hydrogen level, conversion appears to depend on the catalytic effect of FeS, derived from the coal ash. Some deviations from this basic situation are observed in response to temperature and time variables. Higher temperatures tend to lower the hydroaromatic content of the system while rapid feed rates may preclude attainment of equilibrium values (not sufficient time). In addition, higher pressures tend to favor more rapid equilibrium and tend to increase the hydroaromatic character of the system.

In the dissolver stage of the present process, aromatic compounds which have surrendered hydrogen in the preheater are reacted with hydrogen to again form hydroaromatic compounds. Hydroaromatic compounds are partially (not completely) saturated aromatics. The chemical potential in the dissolver is too low for full saturation of aromatics to be a significant reaction. This is important because while hydroaromatics are capable of hydrogen transfer, saturated aromatics are not. Most of the saturates observed in the dissolver tend to be light products derived from ring opening of liquid product or solvent, or derived from aliphatic side chain removal. Solid fuel product aromatic species tend to remain aromatic or hydroaromatic.

This invention is based upon the use of the effect of time in conjunction with the effect of temperature in the preheater stage. It is based upon the discovery that the desired temperature effect in the preheater stage is substantially a short time effect while the desired temperature effect in the dissolver requires a relatively longer residence time. The desired low preheater residence times are accomplished by utilizing an elongated tubular reactor having a high length to diameter ratio of at least 100, generally, and at least 1,000, preferably, so that rapidly upon reaching the desired maximum preheater temperature the preheater stream is discharged and the elevated temperature is terminated by forced cooling. Forced cooling can be accomplished by

hydrogen quenching or by heat exchange. Thereupon, in the dissolver stage, wherein the temperature is lower, the residence time is extended for a duration which is longer than the preheater residence time.

The data in Table 1, show that there is an adverse effect in employing excessively high preheater temperatures.

carbon gas yield above 6 weight percent, while a 450°C. preheater temperature results in a hydrocarbon gas yield below 6 weight percent.

The data of Table 1 show that by far the best result are obtained when the maximum temperature in the preheater is higher than the temperature in the dissolver, provided that the maximum preheater tempera-

TABLE 1

| TEST NUMBER                                                 | 1             | 2             | 3             | 4             | 5             |
|-------------------------------------------------------------|---------------|---------------|---------------|---------------|---------------|
| H <sub>2</sub> Pressure, kg/cm <sup>2</sup>                 | 70            | 70            | 70            | 70            | 70            |
| Max. Preheater Temp., °C.                                   | 450           | 500           | 450           | 450           | 475           |
| Dissolver Temp., °C.                                        | 450           | 450           | 425           | 425           | 425           |
| 1/LHSV; Hr.                                                 | 0.52          | 0.98          | 1.79          | 1.89          | 1.79          |
| GHSV                                                        | 304           | 239           | 342           | 342           | 342           |
| Solvent/MAF Coal/H <sub>2</sub> O (wt)                      | 2.50/1/0.08   | 2.49/1/0.06   | 2.49/1/0.05   | 2.49/1/0.05   | 2.49/1/0.00   |
| % Ash in Feed Slurry                                        | 5.0           | 5.0           | 5.285         | 7.42          | 10.65         |
| % Coal Derived Feed                                         | 33.3          | 33.3          | 34.8          | 48.7          | 69.9          |
| <b>YIELDS ON MAF COAL BASIS-%</b>                           |               |               |               |               |               |
| CO                                                          | 0.23          | 0.42          | 0.51          | 0.27          | 0.28          |
| CO <sub>2</sub>                                             | 1.12          | 1.20          | 0.64          | 0.68          | 0.28          |
| H <sub>2</sub> S                                            | 2.32          | 2.12          | 2.04          | 1.62          | 1.95          |
| Hydrocarbon Gas                                             | 5.28          | 8.89          | 5.73          | 5.80          | 7.11          |
| Gas Not Identified                                          | —             | —             | —             | —             | 12.87         |
| H <sub>2</sub> O                                            | 3.60          | 4.10          | 3.82          | 1.22          | 1.81          |
| Excess Solvent                                              | 5.36          | 15.10         | 31.98         | 62.08         | 49.37         |
| Vacuum Bottoms                                              | 68.12         | 56.81         | 48.66         | 30.36         | 21.06         |
| Insol. Organic Matter                                       | 14.91         | 13.83         | 11.59         | 4.99          | 9.07          |
| <b>TOTAL</b>                                                | <b>100.94</b> | <b>102.47</b> | <b>104.97</b> | <b>107.92</b> | <b>103.20</b> |
| <b>DATA</b>                                                 |               |               |               |               |               |
| Recovery, weight %                                          | 97.94         | 96.59         | 95.91         | 92.63         | 93.35         |
| MAF Conversion, weight %                                    | 85.09         | 86.17         | 88.41         | 95.01         | 90.93         |
| <b>COMPOSITION OF LIQUID AND VACUUM BOTTOM FUEL PRODUCT</b> |               |               |               |               |               |
| Carbon, weight %                                            | 89.68         | —             | 89.40         | 89.72         | 90.65         |
| Hydrogen, weight %                                          | 5.94          | —             | 5.93          | 6.20          | 6.54          |
| Nitrogen, weight %                                          | 0.979         | —             | 1.06          | 1.15          | 1.31          |
| Sulfur, weight %                                            | 0.46          | —             | 0.410         | 0.420         | 0.438         |
| Oxygen, weight %                                            | 4.13          | —             | 5.00          | 2.51          | 1.062         |
| <b>VACUUM BOTTOMS FUEL PRODUCT COMPOSITION</b>              |               |               |               |               |               |
| Carbon, weight %                                            | 87.32         | 89.03         | 88.54         | 88.71         | 91.12         |
| Hydrogen, weight %                                          | 5.11          | 5.12          | 4.74          | 5.35          | 5.10          |
| Nitrogen, weight %                                          | 1.91          | 2.02          | 2.22          | 2.10          | 2.22          |
| Sulfur, weight %                                            | 0.944         | 0.719         | 0.676         | 0.606         | 0.488         |
| Oxygen, weight %                                            | 4.58          | 3.04          | 3.619         | 3.156         | 1.00          |
| Ash, weight %                                               | 0.133         | 0.067         | 0.205         | 0.078         | 0.075         |

As shown in Table 1, an increase in maximum preheater temperature from 450°C. to 475°C. or 500°C., results in an increased yield of hydrocarbon gases to a level above 6 weight percent based on MAF coal feed. A 6 weight percent hydrocarbon gas yield on a MAF basis is a suitable upper limit for gas production unless gas handling facilities are available. Not only are hydrocarbon gases considerably lower economic value than liquid and deashed solid fuel product, but they contain a considerably higher ratio of hydrogen to carbon than either liquid or deashed solid fuel product. Therefore, excessive production of hydrocarbon gases not only signifies a depressed yield of liquid and solid fuel product but also constitutes an unnecessary consumption of valuable process hydrogen due to hydrocracking of higher molecular weight fuel to produce the by-product hydrocarbon gases. Table 1 shows that preheater temperatures of 475°C. and 500°C. both result in a hydro-

ture is below 475°C. (for example, below 470°C.). Table 1 shows that the use of a preheater temperature of 450°C. and a dissolver temperature of 425°C., rather than a temperature of 450°C. in both stages, results in an increase in the ratio of excess solvent (liquid fuel product) yield to vacuum bottoms (solid fuel product) yield, an increase in conversion of MAF coal, and a reduction in the sulfur content of the excess solvent plus vacuum bottoms product and of the vacuum bottoms product itself. These data clearly show the considerable advantages realized by employing a higher temperature at the preheater exit than in the dissolver, as compared to employing a uniform temperature at the preheater exit and in the dissolver, even though the split temperature results in an overall lower average temperature in the process.

The data of Table 1 show that when employing a maximum preheater temperature of 475°C. and a lower

dissolver temperature, the ratio of solvent to vacuum bottoms yield, the percent MAF conversion, the total liquid and vacuum bottoms sulfur content and the vacuum bottoms sulfur content all improved when compared to a test employing a uniform maximum preheater temperature and dissolver temperature, but the improvement is achieved at the expense of excessive hydrocarbon gas yield, which ranged above 6 weight percent. Based upon the data of Table 1, the preheater temperature preferably should not be higher than 460° or 470°C. The preheater effluent should preferably be quenched at least about 25°C. and as much as 50° or 100°C. before entering the dissolver. In some cases a smaller extent of cooling, such as to at least 10°, 15° or 20°C. below the maximum or outlet preheater temperature can be effective.

Test 4 of Table 1 shows an especially advantageous split temperature test of the present invention because the liquid product yield (excess solvent) is greater than the vacuum bottoms yield (solid deashed fuel product)

ing, considerable backmixing occurs in the dissolver which contributes to a uniform temperature throughout the dissolver.

In the dissolver, the reactions occurring require a temperature lower than the maximum preheater temperature. Rehydrogenation of the aromatics in the solvent to replenish hydrogen lost from the solvent by hydrogen donation reactions in the preheater requires a longer residence time than is required in the preheater, 10 but proceeds at a temperature lower than the preheater temperature. After the solvent is hydrogenated in the dissolver to reconver aromatics to hydroaromatics, it is in condition to be recycled to the next preheater pass for hydrogen donation reactions. A coincident reaction 15 which occurs in the dissolver in addition to formation of hydroaromatics is the removal of additional sulfur from the extracted coal. The relatively higher preheater temperatures are more effective for sulfur removal than the lower dissolver temperatures. However, 20 some of the sulfur cannot be removed at the low resi-

TABLE 2

| TEST NUMBER                                 | 1      | 2      | 3      | 4      | 5      |
|---------------------------------------------|--------|--------|--------|--------|--------|
| H <sub>2</sub> Pressure, kg/cm <sup>2</sup> | 70     | 70     | 70     | 70     | 70     |
| Max. Preheater Temp., °C.                   | 450    | 450    | 450    | 450    | 450    |
| LHSV                                        | 28.36  | 28.36  | 28.35  | 15.23  | 7.74   |
| GHSV                                        | 3035   | 2964   | 2953   | 3012   | 3083   |
| 1/LHSV; Hr.                                 | 0.035  | 0.035  | 0.035  | 0.066  | 0.129  |
| YIELDS ON MAF COAL BASIS—%                  |        |        |        |        |        |
| CO                                          | 0.03   | 0.03   | 0.07   | 0.06   | 0.25   |
| CO <sub>2</sub>                             | 0.35   | 0.35   | 0.35   | 0.45   | 0.51   |
| H <sub>2</sub> S                            | 0.94   | 0.97   | 1.73   | 1.49   | 2.66   |
| Hydrocarbon Gas                             | 0.31   | 0.31   | 0.21   | 0.65   | 0.76   |
| H <sub>2</sub> O                            | 0.66   | −1.42  | 1.11   | 0.91   | −0.12  |
| Excess Solvent                              | −38.47 | −59.30 | −39.61 | 7.84   | 11.80  |
| Vacuum Bottoms                              | 65.57  | 136.21 | 105.31 | 75.78  | 69.93  |
| Insoluble Organic Matter                    | 71.06  | 23.20  | 31.34  | 13.21  | 15.23  |
| TOTAL                                       | 100.45 | 100.35 | 100.55 | 100.39 | 101.02 |
| DATA                                        |        |        |        |        |        |
| Recovery, weight %                          | 94.14  | 95.46  | 96.80  | 90.68  | 95.94  |
| MAF Conversion, weight %                    | 28.94  | 76.80  | 68.66  | 86.79  | 84.77  |
| VACUUM BOTTOMS FUEL PRODUCT PROPERTIES      |        |        |        |        |        |
| Carbon, weight %                            | —      | —      | —      | —      | 84.00  |
| Hydrogen, weight %                          | —      | —      | —      | —      | 5.71   |
| Nitrogen, weight %                          | —      | —      | —      | —      | 1.93   |
| Sulfur, weight %                            | —      | —      | —      | —      | 1.38   |
| Oxygen, weight %                            | —      | —      | —      | —      | 6.59   |
| Ash, weight %                               | —      | —      | —      | —      | 0.39   |

and the hydrocarbon gas yield is relatively low.

Higher temperatures can be advantageously employed in the preheater than in the dissolver only in conjunction with a lower residence time in the preheater than in the dissolver. Most of the residence time in the preheater is employed in heating the coal-solvent slurry mixture to the maximum preheater temperature, which is the exit preheater temperature. Preheater reactions are rapid and tend to occur at the required maximum temperature with a low residence time. On the other hand, the reactions which occur in the dissolver are slower reactions. Therefore, the dissolver not only operates at a lower temperature than the maximum preheater temperature but also at a longer residence time. Although the preheater substantially avoids backmix-

55 residence time of the preheater, but requires an extended residence time. Therefore, additional sulfur in the coal product is removed during the extended residence time utilized in the dissolver. A third and highly important reaction occurring in the dissolver is the addition of hydrogen to free radicals formed in both the preheater and the dissolver to arrest polymerization of molecular fragments to high molecular weight material.

Table 2 shows the results of preheater tests which 60 were all conducted at 450°C. Certain of the tests were conducted at a very low preheater residence time of 0.035 hours and other tests were performed at somewhat longer preheater residence times.

As shown in Table 2, at the lowest residence time tests there is a net loss of liquid solvent (due to binding

of the solvent in a gel). Also the percent conversion of MAF coal is low in the low residence time tests. However, at the higher residence times indicated in Table 2 there is a net production of solvent and the percent conversion of MAF coal is considerably higher. Therefore, it is apparent that while excessive preheater residence time is detrimental in that repolymerization will occur (as evidenced by a second increase in Relative Viscosity to a level above 10), a deficiency in residence time in the preheater at a desired preheater temperature is also undesirable in that the process cannot sustain its solvent needs and in that there is inadequate conversion of coal. Solvent will be supplied from an external source only at process start-up, and once the process achieves equilibrium it will satisfy its own solvent requirements and not depend upon an external solvent supply.

The data in Table 3 illustrate the interchangeability of time and temperature in preheater operation.

20

Table 4 shows tests performed at a relatively mild preheater temperature of 450°C. As shown in Table 4, even at the moderate preheater temperature of 450°C., lengthy preheater residence times result in hydrocarbon gas yields above 6 weight percent. Table 4 shows that as preheater residence times increase from about 0.5 to about 1.3 hours at a constant preheater temperature of 450°C. the yield of vacuum bottoms (solid fuel) product gradually decreases while the yield of solvent (liquid fuel) product gradually increases, together with a disadvantageous increase in hydrocarbon gas yield. Although not shown by the data, the hydrogen content of solvent produced at a low residence time is low as compared to solvent produced at a higher residence time at a given temperature, so that solvent produced at a low residence time tends to be of low quality of hydrogen donation in the preheater stage. Table 4 shows that a 450°C. preheater temperature coupled with a low residence time results in a low yield of hydrocarbon

TABLE 3

| TEST NUMBER                                   | 1             | 2             | 3             | 4             | 5             | 6             |
|-----------------------------------------------|---------------|---------------|---------------|---------------|---------------|---------------|
| H <sub>2</sub> Pressure, kg/cm <sup>2</sup>   | 70            | 70            | 70            | 70            | 70            | 70            |
| Max. Preheater Temp., °C.                     | 475           | 475           | 475           | 500           | 500           | 450           |
| LHSV                                          | 27.57         | 13.65         | 7.81          | 28.36         | 7.68          | 7.74          |
| GHSV                                          | 3102          | 3126          | 3095          | 2988          | 3066          | 3083          |
| I/LHSV; Hr.                                   | 0.036         | 0.073         | 0.128         | 0.035         | 0.130         | 0.129         |
| <b>YIELDS ON MAF COAL BASIS-%</b>             |               |               |               |               |               |               |
| CO                                            | 0.14          | 0.36          | 0.25          | 0.17          | 0.13          | 0.25          |
| CO <sub>2</sub>                               | 0.46          | 0.58          | 0.63          | 0.66          | 0.77          | 0.51          |
| H <sub>2</sub> S                              | 1.57          | 2.59          | 2.01          | 1.77          | 2.94          | 2.66          |
| Hydrocarbon Gas Product                       | 0.62          | 1.29          | 3.27          | 1.85          | 5.11          | 0.76          |
| H <sub>2</sub> O                              | -2.43         | 0.29          | 0.63          | -1.50         | 0.64          | -0.12         |
| Excess Solvent (Liquid Fuel Product)          | -11.13        | 13.09         | 17.11         | 13.43         | 25.45         | 11.80         |
| Vacuum Bottoms (Solid Fuel Product)           | 101.97        | 69.57         | 63.15         | 71.17         | 52.56         | 69.93         |
| Insoluble Organic Matter                      | 9.09          | 13.38         | 14.21         | 12.83         | 13.17         | 15.23         |
| <b>TOTAL</b>                                  | <b>100.29</b> | <b>101.15</b> | <b>101.26</b> | <b>100.38</b> | <b>100.77</b> | <b>101.02</b> |
| <b>DATA</b>                                   |               |               |               |               |               |               |
| Recovery, weight %                            | 99.85         | 98.30         | 96.75         | 98.38         | 96.79         | 95.94         |
| MAF Conversion, weight %                      | 90.91         | 86.62         | 85.79         | 87.17         | 86.83         | 84.77         |
| <b>VACUUM BOTTOMS (SOLID FUEL) PROPERTIES</b> |               |               |               |               |               |               |
| Carbon, weight %                              | —             | 84.62         | 84.87         | 86.67         | 88.30         | 84.00         |
| Hydrogen, weight %                            | —             | 5.56          | 5.42          | 5.33          | 4.96          | 5.71          |
| Nitrogen, weight %                            | —             | 1.90          | 2.04          | 1.78          | 2.10          | 1.93          |
| Sulfur, weight %                              | —             | 1.34          | 1.29          | 1.21          | 0.80          | 1.38          |
| Oxygen, weight %                              | —             | 6.23          | 5.42          | 4.90          | 4.19          | 6.59          |
| Ash, weight %                                 | —             | 0.35          | 0.96          | 0.11          | 0.15          | 0.39          |

Table 3 shows a test performed at 475°C. employing the very low preheater residence time of 0.036 hour in which there is a net loss of solvent in the process. The loss is probably caused by the solvent being bonded in a gel with the coal from which the solvent has insufficient time to become disengaged, and from which the solvent cannot be separated by distillation. However, Table 3 shows that at 475°C. there is a net production of solvent in the process when the preheater residence time is increased. Table 3 further shows that if the temperature is increased to 500°C. the residence time can be reduced again while obtaining a high production of solvent in the process.

55 gases. These data illustrating the effect of preheater residence time indicated that with increasing preheater residence time at a preheater temperature of 450°C., there is a continuous conversion of vacuum bottoms (solid fuel) product to solvent (liquid fuel) product, accompanied by a continuous conversion of product to hydrocarbon gases.

60 The data of Table 3 show that at high maximum preheater temperatures of 475° and 500°C. the effect of residence time tends to be greater than at lower preheater temperatures. Table 3 shows that at 475°C. a very low residence time of 0.036 hours resulted in highly incomplete conversion and a loss of solvent in the process. As

the residence time increased at 475°C., conversion increased as indicated by a net production of solvent in the process together with a decrease in vacuum bottoms (solid fuel) yield. Table 3 shows that at 500°C. with a 0.036 hour residence time, the increase in temperature tends to compensate for the low residence time so that there is a net production of solvent in the process, and the yield is increased at 500°C. (accompanied by a decrease in vacuum bottoms yield) by increasing the residence time to 0.130 hour. At a residence time of 0.130 hour a greater solvent yield and a lower vacuum bottoms yield is achieved at 500°C. than at 475°C., except that hydrocarbon gas yield is higher in the 500°C. test. For comparative purposes, Table 3 shows a test conducted at 450°C. and about the same residence time wherein the solvent yield is lower and the vacuum bottoms yield is higher than in the 500°C. test. Furthermore, the 500°C. test performed at 0.130 hour produced a vacuum bottoms product having only 0.8 percent sulfur which is the lowest sulfur level vacuum bottoms product of all the tests of Table 3. However, the 500°C. test at the 0.130 hour residence time shows the amount of vacuum bottoms produced is diminished in favor of not only liquid product but also gaseous product. As the vacuum bottoms level diminishes, it is seen that conversion to gases becomes increasingly favored, and this therefore tends to ultimately limit the extend of conversion of vacuum bottoms to liquid product. However, if facilities are available to collect and purify gaseous product, the high level of hydrocarbon gas production can be advantageously utilized as a commercial fuel.

solid fuel of all the tests of Table 3 (84.6 percent), and this yield is greater than that shown in Tests 3 and 5 because of the relatively low yield of hydrocarbon gases in Test 4.

Comparing Tables 3 and 4, it is seen that a maximum preheater temperature of 450°C. is sufficiently low that lengthy preheater residence times of more than 0.5 hour are required to achieve significantly high yields of excess solvent (liquid fuel product). At higher preheater temperatures of 475° and 500°C., higher excess solvent yields are achieved at lower residence times. Most importantly, at the elevated preheater temperatures of Table 3, excess solvent yield is much more sensitive to slight changes in residence time than at 450°C. At 450°C., large increases in residence time are required to achieve significant increases in solvent yield. Of all the tests in Tables 3 and 4, the combination in Table 3 of a preheater temperature of 500°C. and a preheater time of 0.130 hour achieved the highest solvent yield and the lowest vacuum bottoms yield. The data show that that solvent yield was reduced by one-half at a lower residence time at a preheater temperature of 500°C. and was also reduced by about one-third at about the same residence time but at a lower preheater temperature of 475°, while it was reduced by more than one-half at the same residence time and a still lower preheater temperature of 450°C. It is seen that there is a considerable interdependence between preheater temperature and preheater residence time.

30 An important distinction between 500°C. preheater operation at which the highest solvent yields are achieved as compared with 450°C. temperature pre-

TABLE 4

| TEST NUMBER                                 | 1      | 2      | 3      | 4      | 5      |
|---------------------------------------------|--------|--------|--------|--------|--------|
| H <sub>2</sub> Pressure, kg/cm <sup>2</sup> | 70     | 70     | 70     | 70     | 70     |
| Max. Preheater Temp., °C.                   | 450    | 450    | 450    | 450    | 450    |
| LHSV                                        | 1.96   | 1.91   | 1.34   | 1.09   | 0.74   |
| GHSV                                        | 208    | 225    | 231    | 228    | 235    |
| 1/LHSV; Hr.                                 | 0.510  | 0.524  | 0.746  | 0.917  | 1.351  |
| YIELDS ON MAF COAL BASIS--%                 |        |        |        |        |        |
| CO                                          | 0.21   | 0.18   | 0.47   | 0.25   | 0.37   |
| CO <sub>2</sub>                             | 1.26   | 1.11   | 1.45   | 1.02   | 1.37   |
| H <sub>2</sub> S                            | 1.74   | 2.58   | 1.50   | 2.42   | 2.86   |
| Hydrocarbon Gas Product                     | 4.89   | 3.86   | 6.31   | 5.34   | 8.83   |
| H <sub>2</sub> O                            | 6.00   | 7.08   | 1.81   | 3.75   | 2.30   |
| Excess Solvent (Distillate Fuel Product)    | 6.00   | 11.73  | 14.74  | 16.98  | 18.97  |
| Vacuum Bottoms (Solid Fuel Product)         | 69.78  | 65.02  | 64.36  | 61.32  | 58.83  |
| Insoluble Organic Matter                    | 11.10  | 10.62  | 10.60  | 10.12  | 9.64   |
| TOTAL                                       | 100.98 | 102.18 | 101.24 | 101.20 | 103.17 |
| DATA                                        |        |        |        |        |        |
| MAF Conversion, weight %                    | 88.90  | 89.38  | 89.40  | 89.88  | 90.36  |
| VACUUM BOTTOMS PROPERTIES                   |        |        |        |        |        |
| Carbon, weight %                            | 87.94  | 86.85  | 87.57  | 87.57  | 88.57  |
| Hydrogen, weight %                          | 5.07   | 5.47   | 5.44   | 5.37   | 5.24   |
| Nitrogen, weight %                          | 2.02   | 2.07   | 1.96   | 2.01   | 2.01   |
| Sulfur, weight %                            | 1.04   | 1.01   | 0.85   | 0.80   | 0.70   |
| Oxygen, weight %                            | 3.82   | 4.46   | 4.05   | 4.00   | 3.36   |
| Ash, weight %                               | 0.11   | 0.14   | 0.13   | 0.25   | 0.12   |
| H/C Atomic Ratio                            | 0.346  | 0.379  | 0.373  | 0.368  | 0.355  |

Table 3 indicates that at temperatures as high as 475°C. or 500°C., gas production can exert a limitation on total fuel product (liquid fuel plus solid fuel). Test 4 of Table 3 realized the highest yield of both liquid and

65 heater operation, is that the low temperature operation is not conducive to as rapid polymerization of free radicals produced in the solvation operation. Tables 3 and 4 show that solvent-insoluble organic matter, which

tends to be produced by free radical polymerization in the process and which decreases desired fuel product, tends to be higher in the 500°C. tests than in the 450°C. tests, even though the preheater residence times are very long in the 450°C. tests. Furthermore, very careful control of residence time in the preheater at 500°C. operation is required if plugging of the tubular preheater due to coke formation is to be avoided, which is a less sever problem in 450°C. operation.

Table 4 shows data to illustrate the effect upon product sulfur level when increasing residence time in the preheater at a constant preheater temperature of 450°C.

As shown in Table 4, the percent MAF conversion is substantially maximized at all the residence times tested. However, product sulfur yields advantageously decrease with increasing residence times.

Table 5 shows the results obtained when varying the outlet or maximum preheater temperature without varying total preheater residence time.

during onset of hydrogen transfer. This binding is so tight that the solvent involved in the gel cannot be distilled from the gel at this stage of the reaction. As the temperature of the increment continues to increase 5 along the length of the preheater to a level of about 300°C., hydrogen transfer from the solvent to the coal proceeds further to an extent that the gel is broken and high viscosity hydrocarbon polymer is dissolved out of the coal and enters into solution with the solvent, causing 10 the Relative Viscosity of the solvent solution containing this polymer to decline to a value below 20. With continued flow to a higher preheater temperature region, heteroatom sulfur and oxygen are removed 15 from the dissolved polymer causing the polymer to depolymerize and form free radicals, resulting in a further drop in the viscosity of the solution. Ultimately, the Relative Viscosity drops to a value below 10 generally, or to a value below 5, or even below 2. The free radicals of depolymerized coal will tend to repolymerized 20 under the elevated temperature conditions near the

TABLE 5

| TEST NUMBER                                 | 1       | 2       | 3       | 4       | 5      |
|---------------------------------------------|---------|---------|---------|---------|--------|
| H <sub>2</sub> Pressure, kg/cm <sup>2</sup> | 70      | 70      | 70      | 70      | 70     |
| Max. Preheater Temp., °C.                   | 200     | 300     | 350     | 400     | 450    |
| LHSV                                        | 28.09   | 28.09   | 27.96   | 28.36   | 28.36  |
| GHSV                                        | 2978    | 2978    | 2978    | 2987    | 3035   |
| 1/LHSV: Hr.                                 | 0.035   | 0.035   | 0.036   | 0.035   | 0.035  |
| YIELDS ON MAF COAL BASIS—%                  |         |         |         |         |        |
| CO                                          | 0.00    | 0.00    | 0.00    | 0.24    | 0.03   |
| CO <sub>2</sub>                             | 0.07    | 0.14    | 0.11    | 0.28    | 0.35   |
| H <sub>2</sub> S                            | 0.04    | 0.07    | 0.07    | 0.66    | 0.94   |
| Hydrocarbon Gas Product                     | 0.00    | 0.00    | 0.00    | 0.03    | 0.31   |
| H <sub>2</sub> O                            | -0.95   | 0.25    | 0.35    | 0.87    | 0.66   |
| Excess Solvent (Liquid Fuel Product)        | -153.91 | -172.38 | -134.95 | -129.56 | -38.47 |
| Vacuum Bottoms (Solid Fuel Product)         | 147.91  | 193.61  | 167.60  | 187.58  | 65.57  |
| Insoluble Organic Matter                    | 106.84  | 78.52   | 67.03   | 40.21   | 71.06  |
| TOTAL                                       | 100.00  | 100.21  | 100.21  | 100.31  | 100.45 |
| DATA                                        |         |         |         |         |        |
| Recovery, weight %                          | 95.21   | 118.58  | 27.02   | 92.19   | 94.14  |
| MAF Conversion, weight %                    | -6.84   | 21.48   | 32.97   | 59.79   | 28.94  |

As shown in Table 5, at a constant residence time of 0.035 hour, solvent is consumed due to gel formation at low preheater temperatures. The solvent loss tends to diminish with elevation of preheater temperatures, but even at higher preheater temperatures the employment of extremely low residence times does not permit complete breaking of the gel and release of the solvent. The data of Table 5 show that adequate residence time must lapse to provide a net production of solvent, whereby the process can be self sustaining in solvent. Minimum preheater residence times must be adequate to at least achieve a net production of solvent.

The data in Table 5 illustrate the earlier explanation of rise in Relative Viscosity as the feed slurry begins its transit through the preheater to plug flow. The increase in Relative Viscosity in a stream increment to a value above 20 is due to formation of a gel between the pulverized or ground coal feed and the solvent as the temperature of the coal-solvent slurry starts to rise in the preheater. This gel is caused by the onset of hydrogen donation from the hydroaromatic solvent to the coal and the gel forms by binding of the solvent and coal

preheater exit unless the holding time in the preheater is terminated and the solution temperature is forced to drop. At this time, the preheater stream is withdrawn from the preheater, quenched or otherwise cooled and passed to a lower temperature dissolver stage before the free radicals can repolymerize to an extent that the Relative Viscosity increases again to a value above 10.

Table 6 shows the results of tests conducted with maximum preheater temperatures of 450°C. and 500°C. and with variable preheater residence times.

As shown in Table 6, at the preheater temperature of 450°C. and the low residence time of 0.035 hour, there is a net loss of solvent. Table 6 shows that the preheater is capable of a net production of solvent either by lengthening the residence time at a preheater temperature of 450°C. or by increasing the final preheater temperature to 500°C., without increasing the residence time. Table 6 illustrates the interchangeability of preheater temperature and preheater residence time.

FIGS. 1 through 6 illustrate the effects of varying certain parameters in the process of this invention. FIG. 7 presents a schematic diagram of the present process.

FIG. 1 shows the relationship between percent conversion of MAF coal and maximum preheater temperature at a space time of 0.035 hour. FIG. 1 shows that very high yields are obtained at temperatures of at least 450°C. at a constant low residence time.

FIG. 2 shows percent conversion of MAF coal as a function of residence time in the preheater. FIG. 2 is based on data taken at 450°C. and shows that substantially maximum conversion (above 80 or 85 percent) is achieved very quickly in the preheater and that continuation of preheater holding time for a considerably greater duration has a very small effect on total conversion. Therefore, at a 450°C. preheater temperature, after about 0.05 or 0.1 hour the preheater time is substantially removed as a process factor in regard to conversion.

the preheater and the dissolver at a uniform temperature level, even if the uniform temperature is higher than either temperature of the dual temperature operation. It is important that there is no advantage in regard to sulfur removal in utilizing a higher average but uniform temperature in both the preheater and the dissolver, but better results are obtained with a split temperature wherein the relatively low temperature in the dissolver stage is compensated by a relatively longer residence time.

FIG. 4 shows the fraction of organic sulfur removed from the vacuum bottoms (deashed solid fuel) product versus residence time at various temperatures. As shown in FIG. 4, a high level of sulfur removal is least dependent upon residence time at elevated temperatures while residence time becomes increasingly impor-

TABLE 6

| TEST NUMBER                                  | 1             | 2             | 3             | 4             |
|----------------------------------------------|---------------|---------------|---------------|---------------|
| H <sub>2</sub> Pressure, kg/cm <sup>2</sup>  | 70            | 70            | 70            | 70            |
| Max. Preheater Temp., °C.                    | 450           | 450           | 450           | 500           |
| LHSV                                         | 28.36         | 28.35         | 15.23         | 28.36         |
| GHSV                                         | 2964          | 2953          | 3012          | 2988          |
| 1/LHSV; Hr.                                  | 0.035         | 0.035         | 0.066         | 0.035         |
| <b>YIELDS ON MAF COAL BASIS-%</b>            |               |               |               |               |
| CO                                           | 0.03          | 0.07          | 0.06          | 0.17          |
| CO <sub>2</sub>                              | 0.35          | 0.35          | 0.45          | 0.66          |
| H <sub>2</sub> S                             | 0.97          | 1.73          | 1.49          | 1.77          |
| Hydrocarbon Gas Product                      | 0.31          | 0.21          | 0.65          | 1.85          |
| H <sub>2</sub> O                             | -1.42         | 1.11          | 0.91          | -1.50         |
| Excess Solvent (Liquid Fuel Product)         | -59.30        | -39.61        | 7.84          | 13.43         |
| Vacuum Bottoms (Solid Fuel Product)          | 136.21        | 105.31        | 75.78         | 71.17         |
| Insoluble Organic Matter                     | 23.20         | 31.34         | 13.21         | 12.82         |
| <b>TOTAL</b>                                 | <b>100.35</b> | <b>100.55</b> | <b>100.39</b> | <b>100.38</b> |
| <b>DATA</b>                                  |               |               |               |               |
| Recovery, weight %                           | 95.46         | 96.80         | 90.68         | 98.38         |
| MAF Conversion, weight %                     | 76.80         | 68.66         | 86.79         | 87.17         |
| <b>VACUUM BOTTOMS (SOLID FUEL PROPERTIES</b> |               |               |               |               |
| Carbon, weight %                             | —             | —             | —             | 86.67         |
| Hydrogen, weight %                           | —             | —             | —             | 5.33          |
| Nitrogen, weight %                           | —             | —             | —             | 1.78          |
| Sulfur, weight %                             | —             | —             | —             | 1.21          |
| Oxygen, weight %                             | —             | —             | —             | 4.90          |
| Ash, weight %                                | —             | —             | —             | 0.11          |
| H/C Atomic Ratio                             | —             | —             | —             | 0.369         |

FIG. 3 shows the sulfur content in the deashed coal product as a function of total preheater and dissolver residence time at various maximum preheater temperatures. FIG. 3 shows that residence time exerts a greater effect on sulfur level in the vacuum bottoms product at high temperatures than at low temperatures. FIG. 3 shows that if significant sulfur is to be removed without utilizing relatively high temperatures, a prolonged residence time must accompany low temperature operation. Therefore, the present process employs a dissolver at a relatively low temperature and a relatively long residence time to accomplish a degree of sulfur removal beyond that which is possible in the preheat alone, which operates at a higher temperature at which long residence times are prohibitive due to the onset of hydrocracking. In this manner, a dual temperature process produces a product having a lower sulfur level than the sulfur level that is obtained by operating both

tant to a high level of sulfur removal at lower temperatures. FIG. 4 again illustrates the basis for employing a relatively low temperature dissolver coupled with an extended residence time in cooperation with a relatively high temperature preheater coupled with a relatively short holding time.

FIG. 5 illustrates the relationship of hydrocarbon gas yield to preheater outlet temperature of 0.035 hours and shows that hydrocracking to gases increases rapidly as the temperature is increased above 400°C., and especially above 450°C. The present invention permits the achievement of high conversion without excessive hydrocracking by utilizing a high temperature only for a short duration (preheater stage) followed by a relatively low temperature for a longer residence time (dissolver stage). In this manner, a high conversion is achieved without a high yield of hydrocarbon gases. Production of hydrocarbon gases constitutes a waste of

product and a needless consumption of hydrogen unless gas handling facilities are available.

FIG. 6 illustrates the effect of temperature and residence time on hydrogen consumption and shows that at low residence times hydrogen consumption is not affected by temperature but at higher residence times (above 0.4 or 0.5 hours) hydrogen consumption is affected by temperature. Either low residence times or low temperatures favor low hydrogen consumptions. Therefore, in the present process, a low residence time is employed in the relatively high temperature preheater while a relatively long residence time is employed in the relatively low temperature dissolver.

FIG. 7 shows schematically the process of the present invention. As shown in FIG. 7, pulverized coal is charged to the process through line 10, contacted with recycle hydrogen from line 40 and forms a slurry with recycle solvent which is charged through line 14. The slurry passes through line 16 to preheater tube 18 having a high length to diameter ratio which is greater than 100, generally, and, preferably, greater than 1,000 to permit plug flow. Preheater tube 18 is disposed in a furnace 20 so that in the preheater the temperature of a plug of feed slurry increases from a low inlet value to a maximum temperature at the preheater outlet.

The high temperature effluent slurry from the preheater is then passed through line 22 where it is cooled before reaching dissolver 24 by the addition of cold makeup hydrogen through line 12. Other methods for cooling can include water injection, a heat exchange or any other suitable means. The residence time in dissolver 24 is substantially longer than the residence time in preheater 18 by virtue of the fact that the length to diameter ratio is considerably lower in dissolver 24 than in preheater 18, causing backmixing and loss of plug flow. The slurry in dissolver 24 is at substantially a uniform temperature whereas the slurry in preheater 18 increases in temperature from the inlet to the exit end thereof.

The slurry leaving dissolver 24 passes through line 48 to flash chamber 50 from which lighter overhead stream passes through line 64 to vacuum distillation column 28 while ash-containing heavy fuel is removed as flash residue through line 52 and passed to filter 58. Ash is removed from the flash residue through line 60 while the deashed residue is passed to vacuum distillation column 28 through line 62.

Gases, including hydrogen for recycle, are removed overhead from distillation column 28 through line 30 and are either withdrawn from the process through line 32 or passed through line 34 to scrubber 36 to removed impurities through line 38 and prepare a purified hydrogen stream for recycle to the next pass through line 40.

A distillate liquid product of the process is removed from a mid-region of distillation column 28 through line 42 and recovered as liquid product of the process. Since the process produces sufficient liquid to be withdrawn as liquid fuel product plus sufficient liquid to be recycled as solvent for the next pass, a portion of the liquid product is passed through line 44 for recycle to line 14 to be employed to dissolve pulverized coal in the next pass.

Vacuum bottoms is removed from distillation column 28 through line 46 and passed to moving conveyor belt 54. On conveyor belt 54 the bottoms product is cooled

to room temperature, at which temperature it solidifies. Deashed solid fuel containing as low as ash content as is practical is removed from conveyor belt 54 by a suitable belt scrapper means, as indicated at 56. As shown in FIG. 7, no material is removed from the process between the preheater and the dissolver and all material entering the preheater passes through both the preheater and dissolver before any product separation occurs.

We claim:

1. A process for preparing deashed solid and liquid hydrocarbonaceous fuel from hydrocarbonaceous feed coal containing ash comprising contacting the feed coal with hydrogen and a solvent for the hydrocarbonaceous material in the coal to form a coal-solvent slurry in contact with hydrogen, passing the slurry and hydrogen through a preheater for a residence time between 0.01 and 0.25 hours, said preheater having a length to diameter ratio of at least 100 to inhibit backmixing so that an increment of said slurry gradually increases in temperature in passage through the preheater from a low inlet temperature to a maximum temperature at the preheater outlet, the maximum temperature at the preheat outlet being 400° to 525°C., the viscosity of an increment of the slurry in passage through the preheater increasing initially to a value at least 20 times the viscosity of the solvent alone when each is measured at a temperature of 99°C., the viscosity of the slurry when measured at 99°C. subsequently dropping to a value lower than 10 times the viscosity of the solvent alone when each is measured at 99°C. in continued passage through the preheater, the viscosity of said slurry finally tending to increase to a value greater than 10 times that of the solvent alone when each is measured at 99°C. at the exit temperature of said preheater but the slurry and hydrogen being removed from said preheater after the relative viscosity drops to a value below 10 but before the relative viscosity finally increases to a value of 10, forcing reduction of the temperature of the slurry at least 10°C. to a temperature at which the viscosity of the slurry does not increase to a value above 10 times that of the solvent alone when each is measured at 99°F., passing the cooled slurry to a dissolver maintained at a temperature between 350° and 475°C. and which is below the temperature at the outlet of the preheater, the residence time of the slurry in the dissolver being greater than in the preheater, removing the slurry from the dissolver and separating the slurry into gaseous product, a fraction which is liquid at room temperature and a deashed fraction which is solid at room temperature, recycling hydrogen contained in said gaseous fraction to the preheater, and recycling at least a portion of said liquid fraction as solvent for said preheater step.
2. The process of claim 1 wherein the maximum temperature in the preheater is 425° to 500°C.
3. The process of claim 1 wherein the temperature is the dissolver is 400° to 450°C.
4. The process of claim 1 wherein the forced reduction in temperature between the preheater and dissolver is at least 50°C.
5. The process of claim 1 wherein the preheater length to diameter ratio is at least 1,000.
6. The process of claim 1 wherein the residence time in the preheater is 0.01 to 0.15 hours.
7. The process of claim 1 wherein the dissolver residence time is 0.1 to 3.0 hours.

8. The process of claim 1 wherein carbon monoxide and steam are used together with or in place of hydrogen.

9. The process of claim 1 wherein the yield of deashed solid fuel is 20 to 80 weight percent based on 5 moisture and ash free coal feed.

10. The process of claim 1 wherein the yield of liquid hydrocarbon fuel is above 10 weight percent based on moisture and ash free coal feed.

11. The process of claim 1 wherein the viscosity of 10 the slurry in the preheater falls to a value at least as low as 5 times the viscosity of the solvent alone when each is measured at 99°C.

12. The process of claim 1 wherein the viscosity of the slurry in the preheater falls to a value at least as low as 2 times the viscosity of the solvent alone when each is measured at 99°C.

13. The process of claim 1 wherein said forced temperature reduction is accomplished by injecting makeup hydrogen into the slurry stream.

14. The process of claim 1 wherein said forced temperature reduction is accomplished by cooling the slurry stream in a heat exchanger.

15. The process of claim 1 wherein the gaseous product comprises less than 6 weight percent of hydrocarbon gases based on moisture and ash free coal feed.

\* \* \* \* \*

15

20

25

30

35

40

45

50

55

60

65

UNITED STATES PATENT OFFICE  
CERTIFICATE OF CORRECTION

PATENT NO. : 3,892,654

DATED : July 1, 1975

INVENTOR(S) : Charles H. Wright and Gerald R. Pastor

It is certified that error appears in the above-identified patent and that said Letters Patent are hereby corrected as shown below:

Col. 13, line 8, after "yield" insert --of solvent--.

Signed and Sealed this

*third Day of February 1976*

[SEAL]

*Attest:*

**RUTH C. MASON**  
*Attesting Officer*

**C. MARSHALL DANN**  
*Commissioner of Patents and Trademarks*